

B. SCHWERIN.

MANUFACTURE OF CHEMICALLY PURE SOLUBLE SILICIC ACID.

APPLICATION FILED APR. 18, 1914.

1,132,394.

Patented Mar. 16, 1915.



*Inventor*  
Boris Schwerin

*Witnesses*  
A. M. Troquer.  
W. H. Wakefield

*By* Harry Fenwick Lawrence  
*Attorney*

# UNITED STATES PATENT OFFICE.

BOTHO SCHWERIN, OF FRANKFORT-ON-THE-MAIN, GERMANY, ASSIGNOR TO ELEKTRO-OSMOSE A. G. (GRAF SCHWERIN GESELLSCHAFT), OF FRANKFORT-ON-THE-MAIN, GERMANY, A CORPORATION.

## MANUFACTURE OF CHEMICALLY-PURE SOLUBLE SILICIC ACID.

1,132,394.

Specification of Letters Patent. Patented Mar. 16, 1915.

Application filed April 18, 1914. Serial No. 832,942.

To all whom it may concern:

Be it known that I, BOTHO SCHWERIN, a subject of the German Emperor, and residing at Frankfort-on-the-Main, Germany, have invented certain new and useful Improvements in the Manufacture of Chemically-Pure Soluble Silicic Acid, of which the following is a specification.

The methods hitherto known for making soluble silicic acid do not yield a chemically pure product and the silicic acid can be preserved for a short time only. By the present method there is obtained in a simple manner a chemically pure and permanent silicic acid.

The procedure is as follows: An alkali silicate solution of 5-10 per cent. strength is poured into a diaphragm cell or into the anodic compartment of a suitably constructed diaphragm apparatus. There may be advantageously used as an anode a perforated electrode lying closely against the inner face of the diaphragm wall. The diaphragm thus made is placed in a vessel containing pure water, the cathode being preferably constructed of wire net and lying closely against the outer face of the wall of the cell. The use of electrodes lying closely against the diaphragm wall, particularly for the positive pole, prevents the separation of amorphous silicic acid.

The preparation of silicic acid for medical purposes is carried out with anodes of platinum netting. For technical use on the other hand the operation may be conducted with a suitable lead-antimony anode while a brass wire netting may advantageously serve as cathode. When current is supplied to the electrodes the alkali migrates through the diaphragm into the cathode chamber while soluble silicic acid remains in the anode chamber. There is, however, a loss arising from the fact that this silicic acid also leaves the anode chamber. This fact is the result of the amphoteric character in a colloidal chemical sense generally exhibited by the silicic acid in the anode chamber, and when acid residues are present the silicic acid migrates through the diaphragm toward the cathode. This disadvantage may be avoided by choice of a suitable diaphragm. Thus it is possible to give the diaphragm such a potential that only the alkali migrates through it, the silicic acid remain-

ing in the anode chamber. A diaphragm which has almost zero potential has proven most advantageous. For example one made of a mixture of carborundum and corundum particularly by the process described in U. S. Patent 1,027,004 is suitable.

At the beginning of the operation, the potential may be low, whereas toward the end when the last traces of alkali have to be removed the potential may be raised to say between 60 and 70 volts. The silicic acid is now completely free from alkali residues but still contains traces of acids which (like mineral acids and carbonic acid) are derived from the manufacture of the alkali silicate. In order to separate these constituents also the cathodic purification is succeeded by an anodic purification. The procedure may be as follows: The silicic acid is introduced into a vessel serving as cathode, the anode being surrounded by a diaphragm which may consist advantageously of parchment paper. When current passes, the acid residues migrate through the diaphragm from the cathode chamber into the anode chamber, while the soluble silicic acid does not vary or move out of the cathode chamber. Proportionally with the extent to which the acid residues wander out the potential may be raised so that even the last traces of acid may be quickly separated. The silicic acid thus obtained is quite chemically pure and, when suitably stored, permanent.

In the drawing attached hereto, which is a vertical section of the apparatus which may be employed for carrying out the process disclosed herein, 1 indicates a vessel of any suitable form in which is mounted a cathode 2 surrounding a diaphragm 3 in which is located anode 4. In the use of this particular apparatus diaphragm or cup 3 receives the alkaline silicate and the vessel 1 is filled with water. When the current is passed between the electrodes, the alkali goes through diaphragm 3 into the vessel 1, whereas the soluble silicic acid remains in the diaphragm or cell 3. If the silicic acid is free from traces of alkali this same apparatus may be employed for the anodic purification. For said anodic purification all that is required is to bring the silicic acid, purified as indicated above, into the vessel 1, the diaphragm 3 for this anodic

purification being made of a mixture of carborundum and corundum as set forth in my Patent No. 1,027,004, already mentioned. As the current is passed between the electrodes the silicic acid remaining in the vessel 1 passes through the diaphragm, and chemically pure soluble silicic acid, remains in the vessel 1.

What I claim, is:

- 0 The method of manufacturing chemically pure soluble silicic acid consisting in subjecting to the action of the electric current an alkaline silicate solution in the anode compartment of a cell provided with a diaphragm of such potential as will allow the

migration therethrough of alkali but prevent the migration of silicic acid, and in subsequently subjecting the silicic acid so obtained to the action of the electric current in a cathode compartment of a cell provided with a diaphragm of such potential as will admit of the migration therethrough of acid residues, but prevent migration of the soluble silicic acid.

In testimony whereof I affix my signature 25 in presence of two witnesses.

BOTHO SCHWERIN.

Witnesses:

JEAN GRUND,

CARL GRUND.